

F. T. SMITH,  
PROCESS OF TREATING FOUL SOLUTIONS,  
APPLICATION FILED APR. 2, 1915.

1,276,130.

Patented Aug. 20, 1918.



FIG. 1



FIG. 2



FIG. 3

INVENTOR

Frank T. Smith,  
By Charles J. Martell,  
Atty

# UNITED STATES PATENT OFFICE.

FRANK T. SMITH, OF JAMAICA PLAIN, MASSACHUSETTS.

## PROCESS OF TREATING FOUL SOLUTIONS.

1,276,130.

Specification of Letters Patent. Patented Aug. 20, 1918

Application filed April 2, 1915. Serial No. 18,746.

*To all whom it may concern:*

Be it known that I, FRANK T. SMITH, a citizen of the United States, residing at Jamaica Plain, in the county of Suffolk and State of Massachusetts, have invented new and useful Improvements in the Processes of Treating Foul Solutions, of which the following is a specification.

This invention relates to the treatment of impure solutions of acid and salt, such as the foul solutions of sulfuric acid and copper sulfate arising in copper-refineries and in the winning of metals by leaching. The object of the process is the production of pure solutions of acid and, usually, salt, utilizing the acid and salt of the foul solution. When this process is applied to foul electrolyte from copper refineries it has the additional advantage of simultaneously yielding pure copper, concentrating most of the impurities in a sludge which may be used as a basic flux, and refining low grade metal (black copper or speise) when available.

This process will be described by explaining its application to foul, copper-refinery electrolyte, for which it is especially suited. It consists of the hereinafter described steps which may be modified somewhat in special cases. Instead of a refinery electrolyte, the acid solution of ferrous sulfate obtained in cleaning iron with sulfuric acid may be used.

In the application of the process to copper refinery electrolyte the steps above referred to are as follows:

1. The concentration of copper in the foul solution is reduced by dilution, by plating out copper using low-grade anodes, or, preferably, by treating in the second step as will be explained later.

2. The foul solution is then subjected to electrolysis as follows: It is passed through anode chambers of electrolytic cells containing soluble anodes, while a pure solution of copper sulfate (preferably acidified with sulfuric acid) flows through the cathode chambers. The anode and cathode chambers are separated by diaphragms in order to prevent the solutions from mixing, yet allowing the current of electricity to pass through. A current of electricity enters the cells through anodes, passes from the foul solution, through the diaphragm to the pure solution, and deposits metallic copper on the cathodes.

The conduction of the current through the diaphragms necessitates the passing of hydrogen, copper and other metals, in the form

of ions, from the anolyte to the catholyte. The negative ions move through the diaphragm in the opposite direction, but they may be disregarded. The acid is, relatively, highly dissociated, and the hydrogen ions move about five times as fast as the other ions, consequently, they will move through the diaphragm at the greatest rate. These hydrogen ions replace copper ions deposited on the cathode from the copper sulfate in the catholyte, thereby forming hydrogen sulfate, or sulfuric acid. The hydrogen ions which pass through the diaphragm from the anolyte are replaced by copper ions formed by the dissolving of the anode, thereby forming copper sulfate. When nearly all of the hydrogen ions, (formed by the dissociation of the acid originally present in the foul solution) have migrated out of the anolyte, the anolyte is nearly neutral and is then treated with a precipitant for iron as hereinafter described. It is to be noted that no acid will be formed at the anodes, since these will be soluble.

More copper sulfate is added to the pure solution if it is to be used as electrolyte in the refinery tanks. Usually it will be advisable to replenish this solution with copper sulfate before it becomes too dilute, unless it is to be used for some purpose for which a low concentration of copper is desirable. The foul solution becomes richer in the metals of the anode, mostly copper. The reduction of the concentration of copper in this solution is made before electrolysis, since it was found on experimenting that unless so reduced, the anode becomes coated with copper sulfate crystals before the acidity is lowered sufficiently. The solution is kept warm to allow a higher concentration of copper sulfate, as well as to save power.

It is obvious that as the concentration of the acid in the anolyte diminishes, the other ions take a more prominent part in conduction, and the amount of copper, nickel, and iron passing through the diaphragm with the hydrogen will be considerable if the concentration of acid is to be reduced quite low. The danger of contaminating the pure copper sulfate solution can be eliminated, and the concentration of copper in the foul solution can be reduced by carrying on the purification electrolysis in two stages. First, the foul solution (which has not been subjected to any special treatment) is used as catholyte, and foul solution which has lost

most of its acidity is used as anolyte. The anolyte loses the remaining acid, and copper, nickel and iron to the catholyte. The rate at which copper is deposited from the catholyte is several times greater than the rate at which it gains copper by migration, so that most of the copper can be plated out. The extent of the gain of the catholyte in acid and impurities is too small to be of much consequence. In the second stage of electrolysis, the nearly copperfree solution (foul electrolyte) passes from the cathode chambers of the first series of cells to the anode chambers of the second series, in which it loses most of its acidity. In this series, pure copper sulfate solution is used as the catholyte. Thus, all of the acidity lost by the foul solution is gained ultimately by the pure copper sulfate solution.

3. When the acidity of the foul solution has been reduced sufficiently, it is passed to precipitation tanks where it may be treated with oxids if still slightly acid, and with ferrous sulfate if there is insufficient iron present for the subsequent operations. Air is then blown through the solution to oxidize the ferrous iron (thereby using up any unneutralized acid) and to precipitate basic ferric salts. If the amount of iron remaining in solution is too high, it is completely precipitated with a basic, commercial precipitant for iron, such as powdered limestone, avoiding an excess so that no copper will be precipitated. The solution is kept hot to facilitate hydrolysis and to keep the copper sulfate in solution. The precipitates from these operations consist chiefly of calcium sulfate, ferric hydroxid, basic salts of iron, antimony and bismuth, arsenates and arsenites. They are removed from the solution by filtration or decantation, and may be briqueted or sintered with fine ore or flue dust, since they contain useful basic fluxes.

4. The filtrate contains, principally, sulfates of copper, nickel and perhaps cobalt. When the amount of nickel is moderately low, this solution may be acidified and used in the cathode chambers as described in part two. Otherwise it may be treated with ammonium sulfate, and the nickel crystallized out in the slightly soluble double sulfate of nickel and ammonium, according to the process of Ricketts, as described in U. S. Patent No. 505,846, Oct. 3rd, 1893, to P. D. Ricketts. This would leave the cobalt (and a small amount of nickel and ammonium) in solution, but these would not interfere with its use as electrolyte.

If this process is used, the precipitation of the iron may be accomplished by means of ammonia, thereby forming ammonium sulfate. Nickel ammonium sulfate is rather soluble in hot water, so that the iron, arsenic, etc., can be removed without this double salt

if the solution is kept hot. Or copper sulfate and nickel sulfate may be separated by crystallization, the copper sulfate being used to obtain the required solution of copper sulfate.

This process was specially devised for the treatment of foul solutions of copper sulfate and sulfuric acid produced in the electrolytic refining of copper. It can, however, be applied to other solutions where the production of a neutral solution without wasting acid, or the recovery of acid, is desired. The anodes may be very impure; black copper or even speise may be used. In this case, more copper sulfate will be consumed than is produced in the process, but this salt is quite cheap. The treatment of the anode may be the main object. In any case the hydrogen ions migrate through a diaphragm leaving the slightly dissociated impurities, and replace the metal in the salt at the cathode. The hydrogen of the acid in the foul solution is replaced by metal ions from the anode, the solution becoming nearly neutral enough to allow the economical precipitation of certain impurities.

The invention will now be more fully described, when taken in connection with the accompanying drawings, and the novel features thereof will be pointed out and clearly defined in the claims at the close of this specification.

The invention herein-described, however, does not consist of the apparatus itself and therefore the drawings are diagrammatic.

In the drawings, Figure 1 is a diagram showing the flow of solution under treatment when two cells are employed.

Fig. 2 is a diagram representing the essential features of the cell.

Fig. 3 is a diagram showing the action in the cell.

Referring to the diagram shown in Fig. 1, the foul solution goes through the following steps.

1. It flows from the tank house into the cathode chamber C<sup>1</sup>, cell I, where it is nearly freed from copper.

2. From C<sup>1</sup> to A<sup>2</sup>, cell II, where it loses by migration to the cathode chamber C<sup>2</sup> most of the hydrogen ions, and gains copper by the dissolving of the anode.

3. From A<sup>2</sup> to A<sup>1</sup>, cell I, where it loses most of the remaining hydrogen ions, and gains still more copper.

4. To a tank in which the iron is oxidized and precipitated, together with the arsenic, antimony, and bismuth.

5. Through a filter; or other device to separate the precipitate, to a tank for treatment for nickel.

6. The solution, now containing only copper sulfate, passes to the cathode chamber C<sup>2</sup>, cell II, where it loses copper by deposition on the cathode, and gains acid by mi-

70

75

80

85

90

95

100

105

110

115

120

125

130

gration of hydrogen ions through the diaphragm.

7. The solution, containing copper sulfate and sulfuric acid, goes to the tank house.

Referring to the diagram shown in Fig. 2: The reaction in the anolyte may be represented by the equation:



where M is a divalent metal (copper, nickel or the like). The hydrogen ions pass through the diaphragm to the catholyte where the change may be represented by the equation:



Thus, acid is "consumed" in the anolyte, and formed in the catholyte; more exactly, the hydrogen ions are transferred to the catholyte. The process will usually be more advantageously carried on in two steps, as previously described, but this introduces no new principles.

25 The action in the cell is shown by the diagram in Fig. 3. The hydrogen ions of the impure solution pass through the diaphragm and replace the copper deposited out of the cathode solution. The dissolving of the anode furnishes copper ions which replace the hydrogen ions lost by migration. In other words, copper deposits on the cathode; copper dissolves from the anode;  $H^+$  (to a less extent other ions) migrate as shown by the arrows.

What I claim is:

1. The process of treating impure electrolytes composed of solutions of acid and salts, said process consisting of electrolyzing the impure solution in the anode chamber of an electrolytic cell which contains a soluble anode while a solution of pure copper sulfate flows through the cathode chamber.

45 2. The process of treating impure electrolytes composed of solutions of acid and salts, said process consisting of passing the impure solution through the anode chamber of an electrolytic cell which contains a soluble anode while an acidified solution of pure copper sulfate flows through the cathode chamber, the two chambers being separated from each other by a diaphragm.

3. The process of treating impure electrolytes composed of solutions of acid and salts, said process consisting of passing the impure solutions through the anode chamber of an electrolytic cell which contains a soluble anode while an acidified solution of pure copper sulfate flows through the cathode chamber, the two chambers being separated from each other by a diaphragm, then treating the anolyte with a precipitant

and then removing the precipitates from the solution.

4. The process of treating impure electrolytes composed of solutions of acid and salts, said process consisting of electrolyzing the impure solution in the anode chamber of an electrolytic cell which contains a soluble anode while a solution of pure copper sulfate flows through the cathode chamber, then adding an oxidizing agent and a basic precipitant for iron, then separating the precipitate and treating the solution to leave only pure copper sulfate, then passing the copper sulfate to the cathode chamber of the cell, then passing the solution to a tank house.

5. The process of treating impure solutions of electrolyte, said process consisting of passing the impure solution into the cathode chamber of an electrolytic cell which is divided into an anode and a cathode chamber by a diaphragm, the anode chamber containing a soluble anode, then passing the solution from the cathode chamber of said cell to the anode chamber of a second cell of similar construction to said first cell, and containing a soluble anode, then causing the solution to pass to the anode chamber of the first cell, then causing the solution to pass from the anode chamber of the first cell to a tank, then treating the solution to remove therefrom all except the pure copper sulfate, then passing the copper sulfate to the cathode chamber of the second cell.

6. The process of treating impure solutions of electrolyte, said process consisting of passing the impure solution into the cathode chamber of an electrolytic cell which also contains an anode chamber having a soluble anode, the anode and cathode chambers being separated from each other by a diaphragm, passing the solution from the cathode chamber of said cell to the anode chamber of a second cell of similar construction to said first cell and containing a soluble anode, then causing the portion of the solution which remains in the anode chamber of the second cell to pass to the anode chamber of the first cell, then passing the solution which remains in the anode chamber of the first cell to a tank, and there adding an oxidizing agent and a basic precipitant for iron, then separating the precipitate and treating the solution to leave only pure copper sulfate, then passing the copper sulfate to the cathode chamber of the second cell, then passing the solution of copper sulfate and sulfuric acid to a tank house.

FRANK T. SMITH.

Witnesses:

CHARLES J. MARTELL,  
FRANCOIS FONTAINE.